

# United States Patent

Weil

[15] 3,674,698

[45] July 4, 1972

- [54] **TRANSMITTING PRESSURE IN A HYDRAULIC SYSTEM**

[72] Inventor: **Edward D. Weil, Hastings-on-Hudson, N.Y.**

[73] Assignee: **Stauffer Chemical Company, New York, N.Y.**

[22] Filed: **Feb. 24, 1970**

[21] Appl. No.: **13,782**

[52] U.S. Cl..... **252/78, 252/49.8, 252/49.9,**  
**252/75, 260/966**

[51] Int. Cl. .... **C09k 3/00**

[58] Field of Search ..... **252/78, 75, 49.9, 49.8;**

- |           |         |                      |          |
|-----------|---------|----------------------|----------|
| 2,995,519 | 8/1961  | Shatynski et al..... | 252/78   |
| 3,352,780 | 11/1967 | Groslambert.....     | 252/33.3 |
| 3,384,686 | 5/1968  | Boschan et al.....   | 260/966  |
| 3,428,714 | 2/1969  | Sconce et al.....    | 260/966  |
| 3,432,437 | 3/1969  | Nail.....            | 252/78   |
| 3,436,441 | 4/1969  | Thompson.....        | 260/966  |
| 3,496,107 | 2/1970  | Lima et al.....      | 252/49.9 |

*Primary Examiner*—Leon D. Rosdol

*Assistant Examiner*—Harris A. Pitlick

**Attorney**—Wayne C. Jaeschke, Martin Goldwasser and Daniel S. Ortiz

[57] ABSTRACT

The transmission of pressure in a closed hydraulic system is accomplished by using an effective amount of benzylated and/or styrenated triaryl phosphate.

[ 56 ]

### References Cited

UNITED STATES PATENTS

2,934,501 4/1960 Moreton..... 252/78

## TRANSMITTING PRESSURE IN A HYDRAULIC SYSTEM

## BACKGROUND OF THE INVENTION

Functional fluids suitable for the operation of hydraulic mechanisms require a combination of properties which are often unattainable in many presently available materials. The properties which are required for safe and satisfactory low temperature operation include a low pour point which permits a hydraulic fluid to operate at low temperatures. Another important property which is desirable in hydraulic fluids is a flat viscosity temperature curve, that is, a high viscosity index, which allows the fluid to remain operable over a wide range of temperatures. One of the vital properties which is required for hydraulic fluids which are to be utilized in either commercial industry and mining or military use is minimum flammability. Other desirable qualities for such products include a relatively high boiling point, low corrosion characteristics and low oxidation susceptibility.

It is known in the art that the viscosity index of hydraulic fluids normally decrease when they contain an increasing proportion of cyclic structures. (References: Murphy et al., INDUSTRIAL AND ENGINEERING CHEMISTRY, Vol. 42, page 2,415; Bried et al., INDUSTRIAL AND ENGINEERING CHEMISTRY, Vol. 45, pages 484 and reference cited therein.) Therefore, highly aromatic compounds are usually poor choices for hydraulic fluids. It is also known that benzyl compounds are normally highly susceptible to free radical attack upon the benzyl moiety by oxygen and other reactive species. Therefore, benzylated and styrenated compounds should exhibit low oxidative stability and would therefore be considered to be poor choices for hydraulic fluids.

## TECHNICAL DISCLOSURE OF THE INVENTION

It has now been discovered that the benzylated and styrenated triphenyl phosphates and their halogen derivatives are suitable for use as hydraulic fluids having been found, surprisingly, to possess all the above described properties required for the successful utilization of such products. It has further been discovered that the alpha-methylbenzylphenyl diaryl phosphates and their halogen derivatives are particularly suitable for such usage.

The phosphates employed in the process of the present invention are the benzylated and styrenated triaryl phosphates having the structure:



wherein  $n$  is a number from 0.5 to 2 inclusive,  $m$  is a number between 1 and 3 inclusive,  $x$  is chlorine or bromine,  $R^2$ ,  $R^3$  and  $R^4$  are each a lower alkyl group having from one to about eight carbon atoms,  $a$  and  $d$  are each numbers from 0 to 5 inclusive, such that the sum of  $a$  and  $d$  does not exceed 5,  $b$  is a number between 0 and 4 inclusive,  $c$  is a number from 0 to 5 inclusive,  $R$  and  $R^1$  are each hydrogen or methyl. These compounds can be prepared by the method of U.S. Pat. No. 3,428,714 or by the process described in co-pending application Ser. No. 13,780 filed Feb. 24, 1970 by Edward D. Weil.

Illustrative of these compounds are:

benzylphenyl diphenyl phosphate  
bis(benzylphenyl)phenyl phosphate  
chlorobenzylphenyl diphenyl phosphate  
bis(chlorobenzylphenyl)phenyl phosphate  
pentachlorobenzylphenyl diphenyl phosphate  
bis(pentachlorobenzylphenyl)phenyl phosphate  
pentachlorobenzylphenyl diphenyl phosphate  
bis(alpha-methylbenzylphenyl)phenyl phosphate  
bis(alpha-methylbenzylphenyl)tolyl phosphate  
bis(alpha-methylbenzylphenyl)xylyl phosphate  
bis[di(alpha-methylbenzyl)phenyl]phenyl phosphate  
bis[di(alpha-methylbenzyl)phenyl]tolyl phosphate

bis[tri(alpha-methylbenzyl)phenyl]phenyl phosphate  
bis[tri(alpha-methylbenzyl)phenyl]tolyl phosphate  
bis(alpha-methylbenzyl-4-cresyl)phenyl phosphate  
bis(alpha-methylbenzylphenyl)nonylphenyl phosphate  
bis[di(alpha-methylbenzyl)nonylphenyl]phenyl phosphate  
bis[tri(alpha-methylbenzyl)phenyl] nonylphenyl phosphate  
alpha-methylbenzylphenyl diphenyl phosphate  
alpha-methylbenzylphenyl ditolyl phosphate  
[di(alpha-methylbenzyl)phenyl] dixylyl phosphate  
methylchlorobenzylphenyl diphenyl phosphate  
bis(methylchlorobenzylphenyl)phenyl phosphate  
methylbromobenzylphenyl diphenyl phosphate  
bis(methylbromobenzylphenyl)phenyl phosphate  
alpha-methyl-pentachlorobenzylphenyl diphenyl phosphate  
bis(alpha-methyl-pentachlorobenzylphenyl)phenyl phosphate

and the like, including the various isomers of the compounds.

The preferred compounds for use in the present invention are the alpha-methylbenzyl compounds, that is, those compounds having  $R$  equal to methyl and  $R^1$  equal to hydrogen in the generic formula given above. The use of the latter compounds is preferred because of their high degree of oxidative stability along with their surprisingly high viscosity indices, even as compared with the other compounds coming within the scope of this invention. This is particularly surprising, since the alpha-methylbenzyl compounds would normally be expected to exhibit the lowest oxidative stability of the compounds of the present invention since the alpha-methyl group normally activates a benzyl group toward oxidative attack. Particularly, preferred compounds are:

bis(alpha-methylbenzylphenyl)phenyl phosphate  
alpha-methylbenzylphenyl diphenyl phosphate

and their halogen substituted derivatives where the halogen is attached to the benzyl group(s).

The latter compounds are characterized by having desirable high viscosity indices. This is surprising since they have a large proportion of cyclic structures per molecule which would normally be expected to lower their viscosity indices as was stated above. Thus, one would expect the triaryl phosphates such as the tricresyl and trixylyl phosphates to have higher viscosity indices than the benzylated and styrenated triaryl phosphates of the present invention. However, the compounds of the present invention exhibit viscosity indices which are much higher than those of the triaryl phosphates.

The benzylated and styrenated triaryl phosphates used in the process of the present invention can be used individually or blended with one another, so as to obtain a fluid having properties which are intermediate between the individual phosphates thus blended. The functional fluids of this invention can also contain anticorrosion agents, defoamers and various load bearing additives all of which are well described in the literature. For economic reasons, the functional fluids of this invention can be mixed with less costly petroleum oils and/or polychloroaromatic compounds, particularly polychlorobenzyls and polychlorobiphenyls.

The compounds used in the process of the present invention are deployed in a closed hydraulic system such as a compressor, hydraulic lift, deck edge elevators, basic oxygen furnace, die casting equipment, leveling device or servo control unit in such a manner that when pressure is applied to the phosphate at a specific point within the confines of the hydraulic system, the pressure will be transmitted to any other point along the hydraulic system by the phosphate.

## EXAMPLES

70 Three compounds which are suitable for the process of the present invention were tested along with a commercially available hydraulic fluid which has a triaryl phosphate base and is sold under the name FYRQUEL 220, sold by Stauffer Chemical Chemical of New York. The results of these tests 75 are contained in Tables 1 and 2.

TABLE 1  
Physical Properties

|                                           | Fluid                            |                                             |                                                     |             |
|-------------------------------------------|----------------------------------|---------------------------------------------|-----------------------------------------------------|-------------|
|                                           | Benzyl-phenyl-diphenyl-phosphate | Alpha-methylbenzylphenyl-diphenyl-phosphate | Alpha-alpha-dimethylbenzylphenyl-diphenyl-phosphate | FYRQUEL 220 |
| Viscosity (Saybolt Universal Seconds) at— |                                  |                                             |                                                     |             |
| 100° F.                                   | 174                              | 367                                         | 586                                                 | 212         |
| 210° F.                                   | 42.8                             | 58.4                                        | 56.1                                                | 43.5        |
| Viscosity Index                           | 49                               | 111                                         | 18                                                  | 14          |
| Autoignition temperature                  | 1,150                            | 1,100                                       | 1,076                                               | 1,050       |

From Table 1 it is obvious that the compounds tested are superior to the commercial product in viscosity index and autoignition temperature.

each lower alkyl having from one to about eight carbon atoms, *b* is a number from 0 to 4 inclusive, *c* is a number from 0 and 5 inclusive, *a* and *d* are each numbers from 0 and 5 inclusive,

TABLE 2  
Oxidative Stability

The same samples were tested to determine their ability to resist oxidation (Federal Test Method Std. No. 791a. Method).

|                                   | Fluid                            |                                             |                                                     |             |
|-----------------------------------|----------------------------------|---------------------------------------------|-----------------------------------------------------|-------------|
|                                   | Benzyl-phenyl-diphenyl-phosphate | Alpha-methylbenzylphenyl-diphenyl-phosphate | Alpha-alpha-dimethylbenzylphenyl-diphenyl-phosphate | FYRQUEL 220 |
| Viscosity at 100° F. (S.U.S.) at— |                                  |                                             |                                                     |             |
| 0 hrs.                            | 174                              | 367                                         | 586                                                 | 212         |
| 24 hrs.                           | 175                              | 371                                         | 607                                                 | 221         |
| 48 hrs.                           | 181                              | 372                                         | 617                                                 | 222         |
| 72 hrs.                           | 181                              | 373                                         | 634                                                 | 229         |
| 96 hrs.                           | 189                              | 372                                         | 664                                                 | 232         |
| Change in viscosity, percent      | 8.8                              | 4.2                                         | 11.6                                                | 9.4         |
| Acid number:                      |                                  |                                             |                                                     |             |
| 0 hrs.                            | 0.14                             | 0.09                                        | 0.19                                                | 0.20        |
| 24 hrs.                           | 0.20                             | 0.30                                        | 0.24                                                | 0.92        |
| 48 hrs.                           | 0.50                             | 0.70                                        | 0.42                                                | 1.96        |
| 72 hrs.                           | 0.80                             | 0.70                                        | 1.70                                                | 1.10        |
| 96 hrs.                           | 1.40                             | 0.90                                        | 1.89                                                | 2.10        |
| Change in acid number             | 1.26                             | 0.81                                        | 1.70                                                | 1.90        |

Table 2 demonstrates that the compounds tested have an oxidative stability comparable or superior to the commercial hydraulic fluid. Further, it demonstrates that the alpha-methyl compounds are far superior in oxidative stability and are, therefore, preferred.

The fluids employed in the present invention also perform favorably when tested in a Vickers 104 Vane Pump. During test runs, these fluids exhibit viscosity, color and neutralization characteristics which are equal to or superior to the commercially available hydraulic fluids tested.

What is claimed is:

1. A process for the transmission of pressure in a hydraulic system which comprises deploying within said hydraulic system an effective amount of a phosphate having structure corresponding to the formula:



wherein *n* is a number from 0.5 to 2 inclusive, *m* is a number from 1 to 3 inclusive, *R* and *R*<sup>1</sup> are each selected from the group consisting of hydrogen and methyl, *R*<sup>2</sup>, *R*<sup>3</sup> and *R*<sup>4</sup> are

such that the sum of *a* and *d* is less than or equal to 5, *x* is selected from the group consisting of chlorine and bromine; and applying pressure to said phosphate at any point in said system so as to thereby transmit the thus applied pressure throughout said system through the medium of said phosphate.

2. The process of claim 1, wherein *R* is hydrogen and *R*<sup>1</sup> is methyl.

3. A process for the transmission of pressure in a hydraulic system which comprises deploying within said hydraulic system an effective amount of alpha-methylbenzylphenyl-diphenyl-phosphate, and applying pressure to said phosphate at any point in said system so as to thereby transmit the thus applied pressure throughout said system through the medium of said phosphate.

4. A process for the transmission of pressure in a hydraulic system which comprises deploying within said hydraulic system an effective amount of bis(alpha-methylbenzyl-phenyl) phenyl phosphate and applying pressure to said phosphate at any point in said system so as to thereby transmit the thus applied pressure throughout said system through the medium of said phosphate.